# EUROPEAN PATENT SPECIFICATION

(11) **EP 0 398 600 B1**
(45) Date of publication and mention of the grant of the patent: **09.10.1996**
(21) Application number: 90305114.2
(22) Date of filing: 11.05.1990
(51) Int. Cl.: G03C 1/08, G03C 1/49, G03C 5/305

(54) **Speed and contrast promoted silver halide doped emulsions**
Empfindlichkeits- und kontrastgesteigerte dotierte Silberhalogenidemulsionen
Emulsions à l'halogénure d'argent dopé à sensibilité et contraste augmentés

(30) Priority: 18.05.1989 GB 8911453
(43) Date of publication of application: 22.11.1990
(73) Proprietor: MINNESOTA MINING AND MANUFACTURING COMPANY, St. Paul, Minnesota 55133-3427 (US)
(72) Inventor: Shor, Steven Michael c/o Building 209-2C-08, Minnesota 55144 (US); Hall, Kevin Peter 5 Blacksmiths Way, Hertfordshire (GB); Slater, Sean Dennis 16 Old School Close, Hertfordshire (GB)
(74) Representative: Bowman, Paul Alan

(56) References cited:
- EP-A- 0 267 598
- DE-A- 2 321 401
- DE-A- 3 403 825
- PATENT ABSTRACTS OF JAPAN vol. 8, no. 192 (P- 298)(1629), 4 September 1984; & JP - A - 5979250

## Description

This invention relates to negative-acting silver halide photographic materials and in particular to photographic elements comprising Group VIII metal doped silver halide emulsions associated with a speed and contrast promoting agent which are suitable for use in the photolithographic printing industry and for the development of daylight handleable contact film.

Photosensitive silver halide materials are commonly used in the photolithographic industry to obtain half tone, dot or line, high contrast images.

To increase the contrast of lithographic films it is common practice to dope the silver halide emulsions with contrast promoting agents, among which are the water soluble Group VIII metal salts, such as the trivalent salts of rhodium, ruthenium and iridium. It is known that good results as regards high covering power (which is the ratio between the maximum density obtained after development and the silver halide coverage) and rapid developability (for productivity increase) can be obtained by using fine grained (less than 0.15 µm) and high chloride content silver halide emulsions. It is known that such emulsions which contain a Group VIII metal as a contrast promoting agent may still not have the required contrast, and as the dopant desensitises the emulsion, it may not have the required speed.

One approach to the development of a daylight handleable contact film has been to modify existing daylight duplicating film. Contact films are negative acting materials which are exposed in contact with an original to record a negative image of the original. Duplicating films are positive acting materials which are exposed in contact with an original to produce an identical copy. To produce a duplicating film, the emulsion is chemically fogged, a metal dopant such as rhodium being required for the reversal process as well as for desensitising purposes. For a contact film, the unfogged duplicating emulsion is far too slow for practical use, primarily due to the level of dopant. As stated previously it is advantageous to have the dopant present for contrast enhancement purposes but to increase the speed and also contrast to usable levels a sensitisation step must be introduced. Conventional gold and sulphur sensitisation does confer some extra speed and contrast but European Patent Applications Nos. 267598 and 138200 and British Patent Applications Nos. 2202341 and 2206700 disclose negative-acting rhodium doped emulsions in which the contrast is enhanced by addition of a hydrazine derivative. Such materials are generally too sensitive to be daylight-handleable, and if this property is required, a desensitiser must be added. Various examples of the latter are disclosed, including 2-mercaptobenzimidazole derivatives.

British Patent No. 741228 discloses the use of 4-substituted 3-amino-5-mercapto-4,1,2-triazoles of general formula (I) in which:
R represents other than H,
in photographic constructions. The compounds of formula (I) are said to restrain the formation of chemical fog without seriously affecting the speed, contrast or other properties of the emulsion.

British Patent No. 2573027 discloses the use of compounds of general formulae (II) and (III) in which:
X represents O or S,
Y represents O, S or NH, and,
D represents substituted or unsubstituted carbon atoms to complete a 6 membered ring,
in a photographic construction as anti-bronzing agents. However, within the patent there is no mention of doping of the emulsions.

U.S. Patent No. 1,725,934 discloses the use of thiazole derivatives in silver halide constructions, but as an anti-fogging agent.

The combination of a triazole (IVa) and tetrazaindene (IVb) is known in the photographic art to act as a stabiliser.

DE-A-3403825 discloses a photographic material comprising a support and photographic layers including at least one silver halide emulsion layer which comprises (1) spectrally unsensitised negative silver halide having an average grain size of 0.1 to 0.3µm and containing 80 mole % or more of silver chloride and (2) an organic desensitiser having an anodic polarographic potential and a cathodic polarographic potential which give a positive sum, and said photosensitive material meets at least one of the following requirements:
(a) said emulsion has undergone substantially no chemical ripening;
(b) a spectrally non-sensitising dye capable of absorbing chiefly the rays in the range of from about 500 to 600 nm is contained in at least one of said photographic layers; and
(c) at least one of the following compounds from (i) to (v) is present in said emulsion layer;
   (i) compounds of the general formula (A) in which:
      Z represents a group of carbon atoms necessary for forming a benzene or naphthalene ring which may have a substituent, X represents sulfur atom, selenium atom, oxygen atom, NH, or N-R, R being an alkyl group, A represents a monovalent group bonded to the carbon atom at the position 2 through a carbon atom, sulfur atom, or oxygen atom, and the ring formed by Z may have a substituent provided that any of the substituents present in the general formula (A) does not contain nitro group, sulfo group, or carboxyl group;
   (ii) compounds of the general formula (B) in which:
      X represents sulfur atom, selenium atom, oxygen atom, or N-R₂ group, R₂ represents a lower alkyl group having preferably 1 to 4 carbon atoms, allyl group, or amino group, R₁ represents hydrogen atom, a halogen atom, or a monovalent group (such as, for example, substituted or unsubstituted alkyl group, allyl group, aryl group, thiol group, alkylthio group, arylthio group, aralkylthio group, amidinothio group, hydroxyl group, alkoxy group, aryloxy group, or amino group) which is bonded to the carbon atom at the position 5 through carbon atom, sulfur atom, oxygen atom, or nitrogen atom, and the compound of general formula B does not have a nitro group, sulfo group, or carboxyl group;
   (iii) heterocyclic compounds having a group bonded through a nitrogen atom to the carbon atom adjacent to the nitrogen atom in the ring;
   (iv) 2-mercaptobenzoic acids; and
   (v) 10⁻⁸ to 10⁻⁵ mole of a water-soluble
rhodium salt per mole of silver halide.

JP-59-79250 discloses a silver halide photosensitive material for imagewise exposure containing at least 95 mol % silver chloride prepared in the presence of from 10⁻⁷ to 10⁻² mol rhodium salt per mole of silver halide. It is processed with a developing solution containing a compound represented by general formula I and a compound represented by general formula II or III, and as a developing agent, substantially only p-dihydroxybenzene type developing agent, and more than 0.2 mol/l sulfite ions, and a pH of at least 11. In the formulae, Y is N or methine; Z is N or C; W, W' are each S, 0, or imino; V is H; n is 0 or 1; R₁ is H, lower alkyl, halogen, or nitro; X is -0H , -CONH₂, or the like; and R₂ is H or lower alkyl.

DE-A-23 21 401 discloses a developer solution for the infectious development of silver halide light-sensitive material, which solution comprises a dihydroxybenzene as silver halide developing agents, an alkali, 0.005 to 0.05 mole per litre of free sulphite, a sulphite ion buffer and at least 10 milligrams per litre of the solution of a heterocyclic mercapto compound of the general formula: in which:
Z represents the non-metallic atoms necessary to complete a 5- or 6-membered heterocyclic ring and comprises one or more carbon atom, nitrogen atom, sulphur atom and/or oxygen atom, the heterocyclic ring may be fused to another ring, and the ring or either or the rings may have one or more substituents; X represents a hydrogen atom, a cation or an alkyl group, and n is 1, 2 or 3.

It has now been found that certain groups of compounds, some of which have previously been used as desensitisers, antifoggants, anti-bronzing agents or stabilisers, have a particular utility as speed and contrast promoting agents in Group VIII metal doped, negative-acting silver halide emulsions, the emulsions being chemically-sensitised or otherwise, and being free from hydrazine derivatives.

According to one aspect of the present invention there is provided a photographic element comprising negative-acting silver halide emulsion characterised by the combination of features that the silver halide is doped with from 2.3 x 10⁻⁵ to 10⁻² moles of a Group VIII metal per mole of silver and that the emulsion is associated with one or more speed and contrast promoting agents comprising a compound having a nucleus of one of the following general formulae: (i) to (iv) in which:
Each R¹ independently represents a hydrogen atom or an alkyl group of 1 to 5 carbon atoms, optionally having one or more substituents selected from hydroxyl moieties, carboxyl moieties, alkoxy carbonyl groups of 1 to 5 carbon atoms, cyano moieties, halogen atoms, nitro moieties, amino moieties and aryl groups of up to 10 carbon atoms, wherein the aryl group may be optionally substituted with one or more substituents selected from alkyl groups of 1 to 5 carbon atoms, hydroxyl moieties, carboxyl moieties, alkoxy carbonyl groups of 1 to 5 carbon atoms, cyano moieties, halogen atoms, nitro moieties and amino moieties,
X¹ represents N or CR⁵, where R⁵ represents R¹ (as defined above) or NO₂,
R² represents a hydrogen atom or SR¹ (R¹ is as defined above) but if X¹ is N then R² is SR¹,
Q represents S or NR¹, in which R¹ is as defined above,
R³ represents an amino group or SR¹ in which R¹ is as defined above, and,
Each R⁴ independently represents R¹ as defined above or a halogen atom, a nitro moiety, a cyano moiety, or an alkoxycarbonyl group of 1 to 5 carbon atoms,
the emulsions being free from hydrazine derivatives.
R¹ is preferably a hydrogen atom or a methyl group,
R² is preferably a hydrogen atom or SH,
X¹ is preferably N, -CH, -CCH₃ or -CNO₂,
R³ is preferably SH, SCH₃ or NH₂, and,
R⁴ is preferably hydrogen.

The invention provides a negative-acting photosensitive silver halide material which may be used to obtain black and white half tone, line or dot images for photolithographic purposes. The element preferably comprises a support, having one or more hydrophilic colloidal layers located thereon, in which at least one layer comprises a fine grain, high chloride content and Group VIII metal doped photographic emulsion associated with one or more speed and contrast promoting agents selected from compounds of general formulae (i) to (iv).

The speed and contrast promoting agents need not be present in the emulsion during imaging, but must be associated with the emulsion during development. Thus, the compounds of general formulae (i) to (iv) may be introduced in to the emulsion from a treatment bath or the developer solution. The compounds may be present in the photographic element during imaging and optionally additional compounds present in the developer solution.

Examples of compounds suitable for inclusion as speed or contrast promoting agents are:

Preferably the fine grain, high chloride content and Group VIII metal doped photographic emulsion is associated with one or more speed and contrast promoting agents selected from compounds A to E.

Conventional sulphur and gold sensitisation is known to confer some extra speed and contrast on these high chloride content rhodium doped photographic emulsions but compounds selected from general formulae (i) to (iv) yield greater speed and contrast increases than conventional sensitisation methods and can be used in combination with or without a chemical sensitisation step.

After image wise exposure of the fine grain, high chloride content rhodium doped silver halide emulsion, the material undergoes a photographic processing step comprising an alkaline developing solution wherein the speed and contrast promoting agent is reactively associated with the emulsion. In a further embodiment it is also possible to introduce the speed and contrast promoting agent in the developer solution followed by conventional washing or fixing but it is preferred that the agents are introduced as a precoating addition.

The term fine grain is used in the context of the present invention to refer to silver halide grains having an average grain size of not more than 0.2 µm. High chloride content refers to the emulsion having at least 60% and preferably at least 80% of its total halide molar content consisting of chloride ions. The emulsion is preferably a chlorobromide emulsion wherein the remainder of the halide content comprises bromide ions and a most preferred emulsion comprises 84% silver chloride : 16% silver bromide having a mean silver halide grain size of 0.09µm.

The term Group VIII metal doped refers to the process whereby during precipitation or physical ripening of the silver halide emulsion, salts of one or more Group VIII metals, e.g., trisodium hexachlororhodate (III), disodium pentachlororuthenate (III) and tripotassium hexachloroiridate (III) are present in the solution. The preferred dopants are water-soluble trivalent salts of rhodium. The speed and contrast increasing effect of the compounds of general formulae (i) to (iv) is directly proportional to the level of dopant. The level of doping may be 2.3 x 10⁻⁵ to 10⁻² moles Group VIII metal salt per mole of silver, preferably 10⁻⁴ to 10⁻² moles Group VIII metal salt per mole of silver and most preferably from 10⁻³ to 10⁻² mole Group VIII metal salt per mole of silver.

The amount of the speed and contrast promoting agent added is in the range 10⁻⁴ to 10⁻¹ mole of agent per mole of silver halide but preferably in the range 10⁻² to 5 x 10⁻² mole of agent per mole of silver halide.

The invention will now be described with reference to the following Examples:

### EXAMPLE 1

### Preparation of a Rhodium Doped Silver Halide Emulsion

A silver halide emulsion of 84 mole % chloride and 16 mole % bromide was prepared by the simultaneous addition under constant agitation of water solution B and water Solution C by the double jet technique over a period of 25 minutes to water gelatin Solution A. The compositions A to C were:

### Solution A

| | |
|---|---|
| Water | 833.3g |
| Gelatin | 25g |
| Polyvinylpyrrolidone (K-30) | 6.33g |
| KBr | 0.167ml (1N) |

### Solution B

| | |
|---|---|
| Water | 368g |
| AgNO3 | 170g |

### Solution C

| | |
|---|---|
| Water | 361.3g |
| KC1 | 62.65g (0.84 moles) |
| KBr | 19.04g (0.16 moles) |
| Na₃RhC1₆.12H₂O | 0.200g |

The water gelatin Solution A was kept at a constant temperature of 40°C. Solution B was added at a constant addition rate whilst the addition rate of Solution C was varied to maintain the potential of the emulsion thus formed at a value of 120 ± 5mV (as measured with a specific electrode for Br ions and a reference electrode of the saturated Ag/AgC1 type). The emulsion so prepared, following the removal of soluble salts by the conventional coagulation method, had a mean grain diameter of 0.09µm. The emulsion was then chemically sensitised with sodium gold chloride and sodium thiosulphate. At the end of the chemical sensitisation a speed and contrast promoting agent selected from compounds A to J in a suitable solvent was added to the emulsion before preparation for coating with the addition of additional gelatin, coating surface active agents and formaldehyde hardener.

The emulsion was coated at a silver coating weight of 2.7g Ag/m² onto a polyester support base which was backed with a red antihalation layer.

The resulting films were exposed through a 0-2, 20cm continuous wedge. The exposing lamp was a Violux 1500S UV lamp at a distance of 52 inches from the film plane. The exposed films were developed in 3M RDC^{TM} developer for 20 seconds @ 40°C and fixed in 3M Fix Roll^{TM} Fixer.

The sensitometric data obtained from silver halide coatings made with compounds A to F are illustrated in Table 1 below.

**TABLE 1**

| Sensitometric Data for Films Containing Representative Examples | | | | | | |
|---|---|---|---|---|---|---|
| Compound | Added ** Amount of Compound (mole/mole AgX) | Relative Speed (Log E) | D_{MAX} | Contrast Θ | | Exposure* |
| | | | | A | C | |
| None | - | - | 0.11 | - | - | 200 |
| None | - | -4.43 | 1.26 | 0.4 | - | 2000 |
| A | 10⁻² | -3.46 | 5.1 | 1.5 | 6.0 | 200 |
| B | 2.5x10⁻³ | -3.52 | 5.2 | 1.23 | 6.5 | 200 |
| C | 10⁻² | -3.53 | 3.6 | 1.27 | 5.4 | 200 |
| D | 10⁻² | -3.50 | 4.2 | 1.35 | 5.4 | 200 |
| E | 10⁻² | -3.60 | 5.3 | 1.44 | 6.5 | 200 |
| F | 10⁻² | -3.78 | 2.8 | 0.95 | 2.8 | 200 |

| | | | | | | |
|---|---|---|---|---|---|---|
| * Exposure on a Violux UV lamp (as described previously) | | | | | | |
| ** Generally the amount added to give maximum effect is listed. | | | | | | |

Contrast A is measured between densities 0.07 and 0.17 above Dmin.

Contrast C is measured between densities 0.5 and 2.5 above Dmin.

Each of compounds A to F were dissolved in an appropriate solvent and added at varying levels as a precoating addition to the emulsion. The emulsion used had the composition described previously and had been chemically sensitised with conventional sulphur and gold compounds. When no speed and contrast enhancing compound is added and with conventional exposure and processing the film shows little development, only on extremely long exposures to UV light does any density build up. However, when the compounds of the invention are added, then a dramatic speed and contrast increase is seen.

### EXAMPLE 2

### Effect of Varying the Halide Ratio of the Emulsion

An alternative to the emulsion composition described in Example 1 was tested with Compound A. The emulsion was made following the protocol described previously except the halide ratio was altered from 84 : 16 chloride to bromide to 96 : 4. Very similar results were observed with increases in both speed and contrast.

### EXAMPLE 3

### Effect of Compound A as a Developer Addition

Some digested emulsion (composition as per Example 1) was coated in the standard fashion with no addition of any of the speed or contrast promoting agents. The film was given the standard exposure and processed in RDC developer having some of compound A added. Washing and fixing were carried out in a conventional fashion.

At high levels of A, boosts in speed and contrast were observed but greater effects were noticed when A was added as a precoating addition.

### EXAMPLE 4

### Effect of Varying the Rhodium Dopant Level in the Emulsion

To investigate whether the effect of the compounds of the present invention was also a function of the rhodium dopant level in the emulsion the following emulsions were made and coated as described below:
Emulsion 1 as detailed previously for Example 1.
Emulsion 2 exactly the same as Emulsion 1 except 0.0421g of Na₃RhCl₆.12H₂O was used.
Emulsion 3 exactly the same as Emulsion 1 except 4.21x10⁻³_{g} of Na₃RhCl₆.12H₂O was used.
Emulsion 4 exactly the same as Emulsion 1 except that no rhodium was used.

The exposure was varied depending on the speed of the coated emulsions. The greater the level of rhodium, the slower the film is and hence, a greater exposure period is required. Emulsion 4 was found to be too fast to be exposed by the Violux UV lamp so exposure was conducted with a quartz lamp.

For each emulsion, four coatings were made as described in Table 2.

**TABLE 2**

| Coating Design | Chemically Digested | Compound A* |
|---|---|---|
| I | No | No |
| II | Yes | No |
| III | No | Yes |
| IV | Yes | Yes |

| | | |
|---|---|---|
| *400ml per mole of a 0.325% solution of Compound A. | | |

The following Tables show the increase in speed (measured at a density of 1), toe and shoulder contrast (measured between 0.07 and 0.17 and 0.5 and 2.5 above Dmin respectively) that occurred on addition of Compound A for undigested and chemically sensitised emulsions (i.e. sulphur and gold sensitised).

**TABLE 3**

| Increase in speed (logE) on addition of Compound A | | |
|---|---|---|
| Emulsion | Chemical Sensitisation | |
| | No | Yes |
| 1 | * | + 0.78 highest level of rhodium |
| 2 | * | + 0.55 |
| 3 | +0.8 | + 0.5 |
| 4 | +0.07 | + 0.4 no rhodium |

| | | |
|---|---|---|
| *In these cases the coatings of the undigested emulsion with no Compound A were too slow to be measured using the same exposure level. For emulsion 1 the speed increase is estimated to be > 2logE for the undigested emulsion. | | |

**TABLE 4**

| Increase in toe contrast (O_{A}) on addition of Compound A | | |
|---|---|---|
| Emulsion | Chemical Sensitisation | |
| | No | Yes |
| 1 | * | +2.0 |
| 2 | * | +1.1 |
| 3 | +0.7 | +0.5 |
| 4 | +0.15 | +0.14 |

**TABLE 5**

| Increase in shoulder contrast (O_{C}) on addition of Compound A | | |
|---|---|---|
| Emulsion | Chemical Sensitisation | |
| | No | Yes |
| 1 | * | +9.8 |
| 2 | * | +6.0 |
| 3 | +2.9 | +3.2 |
| 4 | +0.6 | +0.6 |

**TABLE 6**

| Increase in speed (logE) on Chemical Sensitisation | | |
|---|---|---|
| Emulsion | Compound A | |
| | None | Added as a precoating final |
| 1 | - | +0.2 |
| 2 | - | +0.2 |
| 3 | +0.6 | +0.3 |
| 4 | +0.4 | +0.72 |

From Tables 3 - 6 it can be seen that the addition of Compound A causes a large increase in speed to both undigested and chemically sensitised emulsions. The effect is greater for the undigested emulsion and for emulsions containing the higher levels of rhodium dopant.

The same observations hold for the toe and shoulder contrasts (Table 4 and Table 5 respectively).

Table 6 shows the increase in speed (logE) observed on chemical sensitisation when Compound A is added as a precoating addition or not added at all. It can be seen that with no Compound A present, digestion gives a greater increase in speed with increasing levels of rhodium dopant, when Compound A is added as a final the effect of chemical sensitisation decreases with increasing rhodium dopant level i.e. at higher rhodium levels most of the speed increase comes from the addition of Compound A, the digestion step only gives a small further speed increase.

### EXAMPLE 5

### Effect of various Group VIII dopants

An emulsion similar to that in Example 1 was prepared except that the halide ratio was adjusted so that it was 96 mole % chloride 4% bromide emulsion. Seven emulsions were prepared with the following levels of Group VIII transition metal dopants.
Emulsion 1 no dopant.
Emulsion 2 Na₃RhCl₆12H₂O 0.014g per mole of silver.
Emulsion 3 Na₃RhCl₆12H₂O 0.14g per mole of silver.
Emulsion 4 Na₂[RuCl₅(H₂O)] 0.0093g per mole of silver.
Emulsion 5 Na₂[RuCl₅(H₂O)] 0.093g per mole of silver.
Emulsion 6 K₃IrCl₆ 0.013g per mole of silver.
Emulsion 7 K₃IrCl₆ 0.13g per mole of silver.

Once prepared the emulsion was washed and chemically sensitised in the same way as in Example 1. Compound A was then added at a level of 1.95g per mole of silver. The emulsion was then coated onto clear subbed polyester with the conventional coating aids and hardeners at a coating weight of 2.5g Ag/m².

The resulting films were exposed through a 0-4 10cm continuous wedge. The exposing source was a Thiemer Spektra Proof Daylight containing a 1KW Th1007 polymer bulb. The exposed films were developed in 3M RDC developer for 30 seconds at 35°C and fixed in 3M Fix Roll fixer.

The sensitometric data obtained are given in Table 7. Two different coatings of each emulsion were made using the following design:

| Type | Chemical Sensitisation | Compound A |
|---|---|---|
| i) | yes | absent |
| ii) | yes | present |

**TABLE 7**

| Emulsion | Type | Rel. speed/log E | Maximum Density | Contrast | Exposure/Units |
|---|---|---|---|---|---|
| | | | | | |
| 1 | i) | 3.1 | 4.2 | 4.5 | 1 |
| | ii) | 3.2 | 4.2 | 5.3 | 1 |
| | | | | | |
| 2 | i) | 1.9 | 4.4 | 4.6 | 4 |
| | ii) | 2.2 | 4.4 | 12.2 | 4 |
| | | | | | |
| 3 | i) | .3 | 1.3 | - | 4 |
| | ii) | .9 | 4.2 | 9.3 | 4 |
| | | | | | |
| 4 | i) | 2.6 | 2.7 | 0.7 | 4 |
| | ii) | 2.9 | 4.2 | 5.6 | 4 |
| | | | | | |
| 5 | i) | 1.2 | 1.3 | - | 4 |
| | ii) | 1.4 | 4.2 | 2.4 | 4 |
| | | | | | |
| 6 | i) | 2.6 | 4.4 | 4.8 | 4 |
| | ii) | 2.7 | 4.4 | 6.7 | 4 |
| | | | | | |
| 7 | i) | 1.8 | 3.4* | 4.8 | 4 |
| | ii) | 2.1 | 4.3 | 6.7 | 4 |

| | | | | | |
|---|---|---|---|---|---|
| * Strong solarisation noticed. Speed measured at 1.00 above fog. Contrast measured between 0.5 and 2.5 above fog. | | | | | |

Comparison of the results for the rhodium doped Emulsions 2 and 3 with the undoped Emulsion 1 show the significant effect of Compound A. Improvements in speed and contrast are obtained, the magnitude of the improvement related directly to the level of rhodium dopant. A large increase in maximum density is also observed for Emulsion 3. They also show the overall desensitisation effect of rhodium.

For the ruthenium doped Emulsions 4 and 5 improvements in speed and, especially, contrast and maximum density are again obtained on addition of Compound A.

Emulsions 6 and 7 show the effect of iridium doping. There is an overall desensitisation related to the level of dopant (see li) 6i) and 7i). On addition of Compound A speed, contrast and for the heavily doped emulsion maximum density are increased. For Emulsion 7 solarisation is also observed which is eliminated on addition of Compound A.

## Claims

1. A photographic element comprising negative-acting silver halide emulsion characterised by the combination of features that the silver halide is doped with from 2.3 x 10⁻⁵ to 10⁻² moles of a Group VIII metal per mole of silver and that the emulsion is associated with one or more speed and contrast promoting agents comprising a compound having a nucleus of one of the following general formulae: (i) to (iv) in which:
each R¹ independently represents a hydrogen atom or an alkyl group of 1 to 5 carbon atoms, optionally having one or more substituents selected from hydroxyl moieties, carboxyl moieties, alkoxy carbonyl groups of 1 to 5 carbon atoms, cyano moieties, halogen atoms, nitro moieties, amino moieties and aryl groups of up to 10 carbon atoms, wherein the aryl group may be optionally substituted with one or more substituents selected from alkyl groups of 1 to 5 carbon atoms, hydroxyl moieties, carboxyl moieties, alkoxy carbonyl groups of 1 to 5 carbon atoms, cyano moieties, halogen atoms, nitro moieties and amino moieties,
X¹ represents N or CR⁵, where R⁵ represents R¹ (as defined above) or NO₂,
R² represents a hydrogen atom or SR¹ (R¹ is as defined above) but if X¹ is N then R² is SR¹,
Q represents S or NR¹ in which R¹ is as defined above,
R³ represents an amino group or SR¹ in which R¹ is as defined above, and,
each R⁴ independently represents R¹ as defined above or a halogen atom, a nitro moiety, a cyano moiety, or an alkoxycarbonyl group of 1 to 5 carbon atoms, the emulsion being free from hydrazine derivatives.

2. A photographic element as claimed in Claim 1 characterised in that the Group VIII metal dopant is rhodium.

3. A photographic element as claimed in Claim 1 or Claim 2 characterised in that the speed and contrast promoting agent is a compound selected from: and,

4. A photographic element as claimed in any preceding claim characterised in that the silver halide emulsion comprises a support upon which is coated one or more hydrophilic colloidal layers in which at least one layer comprises a fine grain silver halide emulsion having an average grain size of not more than 0.2µm.

5. A photographic element as claimed in Claim 4 characterised in that the silver halide emulsion comprises a chlorobromide emulsion in which silver chloride comprises at least 60% of the total silver halide content.

6. A photographic element as claimed in any preceding claim characterised in that the speed and contrast promoting agent has a concentration of 10⁻⁴ to 10⁻¹ moles per mole of silver halide.

7. A photographic element as claimed in any preceding Claim characterised in that the concentration of Group VIII metal dopant is from 10⁻⁴ to 10⁻² moles dopant per mole of silver halide.

8. A photographic element as claimed in any preceding claim characterised in that the dopant comprises a water soluble trivalent rhodium salt.

9. A photographic element as claimed in any preceding Claim characterised in that the silver halide emulsion is sulphur and gold sensitised.

10. A photographic process which comprises image wise exposing a photographic element comprising negative acting silver halide emulsion doped with from 2.3 x 10⁻⁵ to 10⁻² moles of a Group VIII metal per mole of silver, the emulsion being free from hydrazine derivatives, developing and fixing said exposed element in which one or more speed and contrast promoting agents is associated with the emulsion during development, said agent being selected from compounds having a nucleus of one of the general formulae: in which:
R¹ to R⁴, X¹ and Q are as defined in Claim 1, with the proviso that the developer solution is not suitable for infectious development of silver halide light-sensitive material.

11. A photographic process as claimed in Claim 10 characterised in that the speed and contrast promoting agent:
(i)is present in the emulsion prior to exposure, and/or,
(ii)is introduced into the emulsion after exposure, and/or,
(iii)is present in the developer solution.

12. A developing solution for a photographic element characterised in that the developing solution comprises one or more speed and contrast promoting agents of formula: in which:
R¹ to R⁴, X¹ and Q are as defined in Claim 1, with the proviso the developer solution is not suitable for infectious development of silver halide light-sensitive material.

## Patentansprüche

1. Photographisches Element, umfassend eine negativ wirkende Silberhalogenidemulsion, gekennzeichnet durch die Kombination von Merkmalen, daß das Silberhalogenid mit von 2,3 x 10⁻⁵ bis 10⁻² Mol eines Metalls der Gruppe VIII pro Mol Silber dotiert ist und daß die Emulsion mit einem oder mehreren die Empfindlichkeit und den Kontrast fördernden Mitteln verbunden ist, die eine Verbindung umfassen, die einen Kern einer der allgemeinen Formeln (i) bis (iv) besitzt: in denen:
jedes R¹, unabhängig, ein Wasserstoffatom oder einen Alkylrest mit 1 bis 5 Kohlenstoffatomen bedeutet, der gegebenenfalls ein oder mehrere Substituenten, ausgewählt aus Hydroxygruppen, Carboxygruppen, Alkoxycarbonylresten mit 1 bis 5 Kohlenstoffatomen, Cyanogruppen, Halogenatomen, Nitrogruppen, Aminogruppen und Arylresten mit bis zu 10 Kohlenstoffatomen, besitzt, wobei der Arylrest gegebenenfalls mit einem oder mehreren Substituenten, ausgewählt aus Alkylresten mit 1 bis 5 Kohlenstoffatomen, Hydroxygruppen, Carboxygruppen, Alkoxycarbonylresten mit 1 bis 5 Kohlenstoffatomen, Cyanogruppen, Halogenatomen, Nitrogruppen und Aminogruppen, substituiert sein kann,
X¹ N oder CR⁵ bedeutet, wobei R⁵ R¹ (wie vorstehend definiert) oder NO₂ bedeutet.
R² ein Wasserstoffatom oder SR¹ (wobei R¹ die vorstehende Definition besitzt), bedeutet, aber falls X¹ N ist, R² dann SR¹ bedeutet,
Q S oder NR¹ bedeutet, wobei R¹ wie vorstehend definiert ist,
R³ eine Aminogruppe oder SR¹ bedeutet, wobei R¹ wie vorstehend definiert ist, und
jedes R⁴, unabhängig, R¹, wie vorstehend definiert, oder ein Halogenatom, eine Nitrogruppe, eine Cyanogruppe oder einen Alkoxycarbonylrest mit 1 bis 5 Kohlenstoffatomen bedeutet, und die Emulsion frei von Hydrazinderivaten ist.

2. Photographisches Element nach Anspruch 1, dadurch gekennzeichnet, daß das Metall der Gruppe VIII als Dotierungsmittel Rhodium ist.

3. Photographisches Element nach Anspruch 1 oder 2, dadurch gekennzeichnet, daß das die Empfindlichkeit und den Kontrast fördernde Mittel eine Verbindung ausgewählt aus und ist.

4. Photographisches Element nach einem der vorstehenden Ansprüche, dadurch gekennzeichnet, daß die Silberhalogenidemulsion einen Träger umfaßt, auf den eine oder mehrere hydrophile, kolloidale Schichten aufgetragen sind, wobei mindestens eine Schicht eine Silberhalogenidemulsion mit feinem Korn umfaßt, das eine durchschnittliche Korngröße von nicht größer als 0,2 µm besitzt.

5. Photographisches Element nach Anspruch 4, dadurch gekennzeichnet, daß die Silberhalogenidemulsion eine Chlorbromidemulsion umfaßt, in der Silberchlorid mindestens 60% des gesamten Silbergehalts umfaßt.

6. Photographisches Element nach einem der vorstehenden Ansprüche, dadurch gekennzeichnet, daß das die Empfindlichkeit und den Kontrast fördernde Mittel eine Konzentration von 10⁻⁴ bis 10⁻¹ Mol pro Mol Silberhalogenid besitzt.

7. Photographisches Element nach einem der vorstehenden Ansporüche, dadurch gekennzeichnet, daß die Konzentration des Metalls der Gruppe VIII als Dotierungsmittel von 10⁻⁴ bis 10⁻² Mol Dotierungsmittel pro Mol Silberhalogenid beträgt.

8. Photographisches Element nach einem der vorstehenden Ansprüche, dadurch gekennzeichnet, daß das Dotierungsmittel ein in Wasser lösliches dreiwertiges Rhodiumsalz umfaßt.

9. Photographisches Element nach einem der vorstehenden Ansprüche, dadurch gekennzeichnet, daß die Silberhalogenidemulsion mit Schwefel und Gold sensibilisiert ist.

10. Photographisches Verfahren, umfassend das bildweise Belichten eines photographischen Elements, umfassend eine negativ wirkende Silberhalogenidemulsion, die mit von 2,3 x 10⁻⁵ bis 10⁻² Mol eines Metalls der Gruppe VIII pro Mol Silber dotiert ist, wobei die Emulsion frei von Hydrazinderivaten ist, Entwickeln und Fixieren des belichteten Elements, in dem während der Entwicklung ein oder mehrere die Empfindlichkeit und den Kontrast fördernde Mittel mit der Emulsion verbunden sind, und wobei das Mittel aus Verbindungen ausgewählt ist, die einen Kern der allgemeinen Formeln besitzen: wobei:
R¹ bis R⁴, X¹ und Q wie im Anspruch 1 definiert sind, mit der Maßgabe, daß die Entwicklerlösung nicht für eine infectiöse Entwicklung des lichtempfindlichen Silberhalogenidmaterials geeignet ist.

11. Photographisches Verfahren nach Anspruch 10, dadurch gekennzeichnet, daß das die Empfindlichkeit und den Kontrast fördernde Mittel:
(i) in der Emulsion vor dem Belichten vorhanden ist, und/oder
(ii) nach dem Belichten in die Emulsion eingemischt wird, und/oder
(iii) in der Entwicklerlösung vorhanden ist.

12. Entwicklerlösung für ein photographisches Element, dadurch gekennzeichnet, daß die Entwicklerlösung ein oder mehrere die Empfindlichkeit und den Kontrast fördernde Mittel der Formel: umfaßt, in denen:
R¹ bis R⁴, X¹ und Q wie im Anspruch 1 definiert sind, mit der Maßgabe, daß die Entwicklerlösung nicht für eine infectiöse Entwicklung des lichtempfindlichen Silberhalogenidmaterials geeignet ist.

## Revendications

1. Elément photographique comprenant une émulsion d'halogénure d'argent à caractère négatif caractérisé par la combinaison de caractéristiques que l'halogénure d'argent est dopé avec de 2,3 x 10⁻⁵ à 10⁻² mole d'un métal du Groupe VIII par mole d'argent et que l'émulsion est associée à un ou plusieurs agents favorisant la rapidité et le contraste comprenant un composé comportant un noyau d'une des formules générales suivantes : (i) à (iv) dans lesquelles :
chaque R¹ représente indépendamment un atome d'hydrogène ou un groupe alkyle de 1 à 5 atomes de carbone, comportant éventuellement un ou plusieurs substituants choisis parmi les fragments hydroxyle, les fragments carboxyle, les groupes alcoxy carbonyle de 1 à 5 atomes de carbone, les fragments cyano, les atomes d'halogène, les fragments nitro, les fragments amino et les groupes aryle jusqu'à 10 atomes de carbone, le groupe aryle pouvant être éventuellement substitué par un ou plusieurs substituants choisis parmi les groupes alkyle de 1 à 5 atomes de carbone, les fragments hydroxyle, les fragments carboxyle, les groupes alcoxy carbonyle de 1 à 5 atomes de carbone, les fragments cyano, les atomes d'halogène, les fragments nitro et les fragments amino,
X¹ représente N ou CR⁵, R⁵ représentant R¹ (tel que défini ci-dessus) ou NO₂,
R² représente un atome d'hydrogène ou SR¹ (R¹ est tel que défini ci-dessus) mais si X¹ est N, alors R² est SR¹,
Q représente S ou NR¹, R¹ étant tel que défini ci-dessus,
R³ représente un groupe amino ou SR¹, R¹ étant tel que défini ci-dessus, et
chaque R⁴ représente indépendamment R¹ tel que défini ci-dessus ou un atome d'halogène, un fragment nitro, un fragment cyano ou un groupe alcoxy carbonyle de 1 à 5 atomes de carbone, l'émulsion étant exempte de dérivés d'hydrazine.

2. Elément photographique suivant la revendication 1, caractérisé en ce que le dopant de métal du Groupe VIII est le rhodium.

3. Elément photographique suivant l'une ou l'autre des revendications 1 et 2, caractérisé en ce que l'agent favorisant la rapidité et le contraste est un composé choisi parmi : et

4. Elément photographique suivant l'une quelconque des revendications précédentes, caractérisé en ce que l'émulsion d'halogénure d'argent comprend un support sur lequel sont appliquées une ou plusieurs couches colloïdales hydrophiles dans lesquelles au moins une couche comprend une émulsion d'halogénure d'argent à grain fin ayant une taille de grain moyenne ne dépassant pas 0,2 µm.

5. Elément photographique suivant la revendication 4, caractérisé en ce que l'émulsion d'halogénure d'argent comprend une émulsion de chlorobromure dans laquelle le chlorure d'argent constitue au moins 60 % de la teneur en halogénure d'argent totale.

6. Elément photographique suivant l'une quelconque des revendications précédentes, caractérisé en ce que l'agent favorisant la rapidité et le contraste a une concentration de 10⁻⁴ à 10⁻¹ mole par mole d'halogénure d'argent.

7. Elément photographique suivant l'une quelconque des revendications précédentes, caractérisé en ce que la concentration de dopant de métal du Groupe VIII est de 10⁻⁴ à 10⁻² mole de dopant par mole d'halogénure d'argent.

8. Elément photographique suivant l'une quelconque des revendications précédentes, caractérisé en ce que le dopant comprend un sel de rhodium trivalent soluble dans l'eau.

9. Elément photographique suivant l'une quelconque des revendications précédentes, caractérisé en ce que l'émulsion d'halogénure d'argent est sensibilisée au soufre et à l'or.

10. Procédé photographique qui comprend l'exposition selon un mode de formation d'une image d'un élément photographique comprenant une émulsion d'halogénure d'argent à caractère négatif dopée avec de 2,3 x 10⁻⁵ à 10⁻² mole d'un métal du Groupe VIII par mole d'argent, l'émulsion étant exempte de dérivés d'hydrazine, le développement et la fixation de l'élément exposé susdit dans lequel un ou plusieurs agents favorisant la rapidité et le contraste sont associés avec l'émulsion au cours du développement, l'agent précité étant choisi parmi les composés comportant un noyau d'une des formules générales : dans lesquelles :
R¹ à R⁴, X¹ et Q sont tels que définis dans la revendication 1, à la condition que la solution de révélateur ne convienne pas pour un développement infectieux de matériel photosensible à halogénure d'argent.

11. Procédé photographique suivant la revendication 10, caractérisé en ce que l'agent favorisant la rapidité et le contraste :
(i) est présent dans l'émulsion avant l'exposition, et/ou,
(ii) est introduit dans l'émulsion après l'exposition, et/ou,
(iii) est présent dans la solution de révélateur.

12. Solution de développement pour un élément photographique, caractérisée en ce que la solution de développement comprend un ou plusieurs agents favorisant la rapidité et le contraste des formules : dans lesquelles :
R¹ à R⁴, X¹ et Q sont tels que définis dans la revendication 1, à la condition que la solution de révélateur ne convienne pas pour un développement infectieux de matériel photosensible à halogénure d'argent.
